

May 19, 1936.

C. E. HEUSSNER

2,041,545

CORROSION RESISTING COATING

Filed May 29, 1933



INVENTOR.  
CARL E HEUSSNER.

BY *John Barnes*  
ATTORNEYS.

## UNITED STATES PATENT OFFICE

2,041,545

## CORROSION RESISTING COATING

Carl E. Heussner, Detroit, Mich., assignor to  
 Chrysler Corporation, Detroit, Mich., a corpora-  
 tion of Delaware

Application May 29, 1933, Serial No. 673,475

## 14 Claims. (Cl. 148—6)

This invention relates to an improved coating for metal articles and to an improved coating bath and method of forming such coatings.

One of the main objects of the invention is to provide a corrosion resisting coating for articles which consist of or contain zinc, such as zinc die cast parts, and particularly to provide a coating of this character which resists corrosion of such articles by halogen and/or sulphur containing salts and acids, mineral and organic acids and the corrosive constituents of motor oils and fuels.

Other objects of the invention are to provide a coating of this character which is smooth and particularly adapted for the reception of plated deposits, such as nickel and chromium, as well as for the reception of paint and enamel; to provide a coating for articles consisting of or containing zinc which renders those portions of such articles upon which metal is not deposited during plating, passive to the corrosive action of the plating bath; and to provide a coating of this kind which is particularly adapted to protect those surfaces of such articles which, due to lack of throwing power of nickel plating solutions, do not receive a nickel coating, so as to prevent corrosion of such surfaces by the solution and contamination of the solution by the corrosion reaction products.

Further objects of my invention are to provide an improved method for coating articles consisting of or containing zinc by which some of the zinc at the exposed surfaces of such articles is caused to react with ingredients of a coating forming bath in such a manner as to form complex salts of zinc and other metals, such as alkaline earth metals and metals selected from the group consisting of manganese and aluminum; to provide a process of this character by which the formation of such compositions is conducted at the surfaces of the articles so as to cause the compositions to become integrally united with the articles; and to provide an improved bath for forming such protective coatings which is stable and from which the contents are not precipitated during operation.

The drawing is a fragmentary sectional view of an article having my improved coating on one side thereof.

My improved corrosion-resisting treatment is particularly adapted for protecting the surfaces of metal articles which either contain or consist of zinc but it may be used to advantage upon articles formed of other non-ferrous metals, as well as ferrous metals. In general, the plating

bath comprises a solution which may be formed by introducing into a suitable quantity of water proper amounts of a nitrate of an alkaline earth metal, a soluble salt of a metal selected from the group of metals consisting of manganese and aluminum, preferably a bivalent metal thereof, and an acidifying agent. The following formulas represent some of the combinations of the above materials which have been found to produce satisfactory results, the proportions set forth being 10 variable within substantially wide limits.

|                      |          |    |
|----------------------|----------|----|
| 1. Barium nitrate    | 15 grams |    |
| Manganous carbonate  | 8 grams  |    |
| Phosphoric acid      | 20 grams | 15 |
| Water                | 1 litre  |    |
| 2. Strontium nitrate | 12 grams |    |
| Manganous carbonate  | 8 grams  |    |
| Phosphoric acid      | 20 grams |    |
| Water                | 1 litre  | 20 |
| 3. Barium nitrate    | 15 grams |    |
| Manganous carbonate  | 8 grams  |    |
| Oxalic acid          | 25 grams |    |
| Water                | 1 litre  | 25 |
| 4. Strontium nitrate | 12 grams |    |
| Manganous carbonate  | 8 grams  |    |
| Oxalic acid          | 25 grams |    |
| Water                | 1 litre  |    |
| 5. Barium nitrate    | 15 grams | 30 |
| Manganous hydroxide  | 8 grams  |    |
| Phosphoric acid      | 20 grams |    |
| Water                | 1 litre  |    |
| 6. Strontium nitrate | 12 grams | 35 |
| Manganous hydroxide  | 8 grams  |    |
| Phosphoric acid      | 20 grams |    |
| Water                | 1 litre  |    |
| 7. Barium nitrate    | 15 grams | 40 |
| Manganous hydroxide  | 8 grams  |    |
| Oxalic acid          | 25 grams |    |
| Water                | 1 litre  |    |
| 8. Barium nitrate    | 15 grams | 45 |
| Aluminum hydrate     | 10 grams |    |
| Phosphoric acid      | 14 grams |    |
| Water                | 1 litre  |    |

From the foregoing formulas it should be understood that strontium nitrate may be used in place of barium nitrate and that oxalic acid may be used in place of phosphoric acid and that either manganous hydroxide or aluminum hydrate may be used in place of manganous carbonate in all of the various combinations. When

oxalic acid is employed it is advantageous, though not necessary, to add a small amount of glucose or dextrose. The addition of  $\frac{1}{2}$  gram of sodium dichromate to any of the above mentioned formulas has been found to be beneficial in the formation of protective coatings upon articles of various metallic compositions.

My improved protective coating forming bath is preferably contained in a lead lined tank or receptacle which is provided with steam heating coils or other heating means capable of maintaining the bath at a temperature of 150 to 212° F. Operation at a temperature of 200° F. or any temperature slightly below the boiling point of water is particularly efficient inasmuch as the chemical action of the contents of the bath upon the article treated is expedited without excessive vaporization of the bath. The articles are preferably cleaned with any commercial cleaning solution, water washed, and then moved through the bath by a conveyer which is operated in such a manner as to allow each article to remain in the bath for from 5 to 15 minutes. When the temperature of the bath is substantially 210° F. a 10 minute treating period is ample to produce a coating of sufficient thickness to protect the article from corrosion.

Protective coatings formed in accordance with my invention include complex salts of the metals introduced into the solution from which they are formed. Some of these salts comprise inorganic compounds having a metal element of the alkaline earth group and a metal element of the aluminum-zinc group combined with the acid radical of phosphoric acid, oxalic acid, or other acids, depending upon which is used as the acidifying agent of the bath. When Formula #1 is employed the resulting coating contains zinc-barium phosphate, manganous barium phosphate, zinc-pyro phosphate, and zinc phosphate, as well as the phosphates of the individual metals of the coating bath. The coatings resulting from solutions having various other compositions set forth above include the complex salts and the salts of the individual metals contained in the bath solution from which they are formed.

A coating formed in accordance with my invention upon articles containing or consisting of zinc is extremely smooth and has the appearance of gunmetal. Such coatings form a suitable under layer for the reception of paints, varnishes, lacquers and enamels, as well as for the reception of metallic plated deposits. Those portions of articles which are so disposed that plating is not deposited thereon due to the lack of throwing power of various plating solutions, such as nickel solutions, are protected from corrosion by the action of the plating bath thereon during plating operations. In this manner fouling of the bath by the corrosion reaction products is practically eliminated.

Although but several specific embodiments of my invention are shown, it is understood that various changes in the materials employed and in the sequence of steps, as well as in the temperature and periods of treatment, may be made without departing from the spirit of my invention, and it is not my intention to limit its scope other than by the terms of the appended claims.

What I claim is:

1. A bath for forming a corrosion resisting coating on articles containing zinc comprising a water solution substantially free from iron and its compounds including the reaction products of

barium nitrate, a water soluble manganous salt, and an acidifying agent.

2. A bath for forming a corrosion resisting coating on zinc and its alloys comprising a water solution substantially free from iron and its compounds having a solute including the reaction products of a nitrate of a metal selected from the group of metals consisting of barium and strontium, a compound selected from the group of compounds consisting of manganous carbonate, manganous hydroxide and aluminum hydrate and an acid selected from the group of acids consisting of phosphoric acid and oxalic acid.

3. The method of forming a corrosion resisting coating on zinc and zinc alloy articles which consists in reacting upon the zinc at the surface of said articles a water solution substantially free from iron and its compounds into which has been introduced a nitrate of a metal selected from the group of metals consisting of barium and strontium; a compound selected from the group of compounds consisting of manganous carbonate, manganous hydroxide and aluminum hydrate and an acid selected from a group of acids consisting of phosphoric acid and oxalic acid.

4. An article formed of metal selected from a group of metals consisting of zinc and zinc alloys having a coating formed thereon substantially free from iron and its compounds including the reaction product of zinc; a nitrate of a metal selected from the group of metals consisting of barium and strontium, a compound selected from the group of compounds consisting of manganous carbonate, manganous hydroxide and aluminum hydrate; and an acid selected from the group of acids consisting of phosphoric acid and oxalic acid.

5. A bath for forming corrosion resisting coatings on zinc and its alloys comprising a water solution substantially free from iron and its compounds having a solute including the reaction products of barium nitrate, manganous carbonate and phosphoric acid.

6. The method of forming a corrosion resisting coating on zinc and zinc alloy articles, which consists in reacting upon the zinc at the surface of said articles a water solution substantially free from iron and its compounds into which has been added barium nitrate, manganous carbonate and phosphoric acid.

7. An article formed of metal selected from a group of metals consisting of zinc and zinc alloys having a coating thereon including a reaction product of some of the zinc of said article, barium nitrate, manganous carbonate and phosphoric acid.

8. A bath for forming corrosion resisting coatings on zinc and zinc alloys comprising a water solution substantially free from iron and its compounds having a solute including the reaction products of a nitrate of a metal selected from the group of metals consisting of barium and strontium, manganous carbonate and an acid selected from a group of acids consisting of phosphoric acid and oxalic acid.

9. A bath forming corrosion resisting coatings on zinc and its alloys comprising a water solution substantially free from iron and its compounds having a solute including the reaction products of barium nitrate, manganous carbonate and oxalic acid.

10. An article formed of metal selected from a group of metals consisting of zinc and zinc alloys having a coating thereon including a reaction

- product of some of the zinc of said article, barium nitrate, manganous carbonate and oxalic acid.
11. The method of forming a corrosion resisting coating on zinc and zinc alloy articles, which consists in reacting upon the zinc at the surface of said articles a water solution substantially free from iron and its compounds into which has been added barium nitrate, manganous carbonate and oxalic acid.
12. A bath for forming corrosion resisting coatings on zinc and its alloys comprising a water solution substantially free from iron and its compounds having a solute including the reaction products of barium nitrate, aluminum hydrate and phosphoric acid.
13. An article formed of metal selected from a group of metals consisting of zinc and zinc alloys having a coating thereon including a reaction product of some of the zinc of said article, barium nitrate, aluminum hydrate and phosphoric acid.
14. The method of forming a corrosion resisting coating on zinc and zinc alloy articles, which consists in reacting upon the zinc at the surface of said articles a water solution substantially free from iron and its compounds into which has been added barium nitrate, aluminum hydrate and phosphoric acid.

CARL E. HEUSSNER. 15